# EUROPEAN PATENT SPECIFICATION

(11) **EP 1 888 815 B1**
(45) Date of publication and mention of the grant of the patent: **18.09.2013**
(21) Application number: 05823699.3
(22) Date of filing: 20.10.2005
(51) Int. Cl.: C23F 11/00, C23C 22/03

(54) **ORGANIC COMPOUND AND PROCESS FOR INHIBITING CORROSION ON METALLIC SURFACES**
ORGANISCHE VERBINDUNG UND VERFAHREN ZUR KORROSIONSINHIBIERUNG VON METALLISCHEN OBERFLÄCHEN
COMPOSÉ ORGANIQUE ET PROCÉDÉ POUR INHIBER LA CORROSION SUR DES SURFACES MÉTALLIQUES

(30) Priority: 13.05.2005 IN MU05812005
(43) Date of publication of application: 20.02.2008
(73) Proprietor: Kelkar, Anil, Pashan, Pune 411008 (IN)
(72) Inventor: Kelkar, Anil, Pashan, Pune 411008 (IN)
(74) Representative: Richards, John
(86) International application number: PCT/IN2005/000342
(87) International publication number: WO 2006/120694

(56) References cited:
- EP-A- 0 651 074
- EP-A- 0 818 651
- DE-A1- 3 711 611
- GB-A- 625 297
- GB-A- 2 104 897
- US-A- 3 397 150
- US-A- 3 846 071
- US-A- 5 611 992
- US-A- 5 960 878
- US-A- 6 135 207

## Description

### TECHNICAL FIELD OF THE INVENTION

The present invention is a process to prepare an organic compound to reduce corrosion on metal surface and the compound obtained there-from. The present invention is a process which displaces primary embedded corrosion, dehydrates water and donates antistatic properties by forming a compact corrosion film with chemi-adsorbed organic compound bond to reduce the rate of corrosion at a very low cost.

### BACKGROUND OF THE INVENTION

Any metal article, produced or manufactured, always has primary embedded corrosion being integral to the environment, f the metal surface. This primary embedded corrosion creates an environment, which is conducive to the growth of corrosion rate.

Primary surface oxide i.e.. Iron oxide is present on the metal surfaces even at the time of manufacturing. This primary surface oxide can be classified into saturated and unsaturated oxide. Any metal when manufactured has primary embedded corrosion due to this saturated oxide. For example, construction steel like rebar used in reinforced cement concrete, when manufactured by any process, has embedded corrosion on the surface. The unsaturated oxide is responsible for growth of corrosion on metal and its alloys. Being unsaturated it does not require any additional donor from the environment, as the donor exist on the metal itself. Exposure to industrial environment, storage, transportation etc. lead to further growth of metal oxidation and corrosion. This increased corrosion and metal oxidation leads to loss of metal, dimension control and surfaced quality requirements of the ferrous material.

There is neither any standard method available to remove the unsaturated oxide nor any method that quarantines such unsaturated oxides so as to selectively control the growth rate of metal loss due to unsaturated oxides.

It is therefore the object of the present invention to selectively control and reduce the rate of corrosion by quarantining such unsaturated oxides from the metal surfaces.

The present invention, therefore, displaces primary embedded corrosion, dehydrates water from the unsaturated oxide and donates anti static properties to reduce the rate of corrosion.

### PRIOR ART

In prior art there exist no processes or methods that selectively deal with the removal of the unsaturated oxides from metal surface to stop further corrosion growth rate and metal loss. Nonetheless there are various methods that deal with the removal of corrosion by varied means.

### References:

1. NATCO Group publication.
2. US 4816303
3. DE3828489 - Process for producing corrosion-inhibiting oxide layers

### NATCO Group publication:

In aqueous systems, there are two basic ways to inhibit corrosion: -
- Remove the corrosive oxygen from the water, either by mechanical or chemical de-aeration.
- Add corrosion inhibitors.

### Corrosion inhibitors

A corrosion inhibitor is any substance, which effectively decreases the corrosion rate when added to an environment.
- Passivating (anodic) inhibitors form a protective oxide film on the metal surface. They are the best inhibitors because they can be used in economical concentrations, and their protective films are tenacious and tend to be rapidly repaired if damaged.
- Precipitating (cathodic) inhibitors are simply chemicals which form insoluble precipitates that can coat and protect the surface

Adsorption inhibitors have polar properties, which cause them to be adsorbed on the surface of the metal. They are usually organic materials.

### Passivation inhibitors

Examples of passivators (anodic inhibitors) include chromate, nitrite, molybdate, and orthophosphate. All are oxidizers and promote passivation by increasing the electrical potential of the iron. Chromate and nitrite do not require oxygen and thus can be effective.

### Precipitating inhibitors

Orthophosphate is a good example of a precipitating inhibitor, which exhibits a dual mechanism, acting as both an anodic passivator and a cathodic precipitator.

### Copper corrosion inhibitors

The most effective corrosion inhibitors for copper and its alloys are the aromatic triazoles, such as benzotriazole (BZT) and tolyltriazole (TTA). These compounds bond directly with cuprous oxide at the metal surface, forming a "chemisorbed" film.

### Adsorbtion inhibitors

Adsorption inhibitors must have polar properties in order to be adsorbed, such as amines. Often, these molecules have dual functionality. They contain a hydrophilic group, which adsorbs onto the metal surface and an opposing hydrophobic group, which prevents further wetting of the metal.

### Silicates

For many years, silicates have been used to inhibit aqueous corrosion, particularly in potable water systems. Their mechanism of inhibition has not yet been firmly established. They appear to inhibit by an adsorption mechanism. Silicates are slow-acting inhibitors, in some cases, 2 or 3 weeks may be required to establish protection fully.

### US 4816303

In yet another prior art, corrosion of ferrous metal and aluminum surfaces, in particular, is inhibited by a layer of an organic-metallic complex of a polyamine with a (i) metal oxide, or (ii) metallate ion, or (iii) water-soluble metallate salt, in aqueous systems having a pH greater than about 7. The polyamine contains at least four (4) amine groups, two of which are secondary amine groups. The effect of the N atoms stretched over the length of the polyamine produces a "caging effect"0 which immobilizes the oxide, or metallate ions, thus forming the protective layer. The organic-metallic complex deposited on the metal's surface forms the "amine-metallic" layer, which may be either an "amine-metal oxide complex" which is a coordination complex, or, an "amine-metallate complex". The amine-metallate complex may be either an ionic complex of "amine metallate ions", or, a mixture of the polyamine and metallate salt which mixture is not a complex, but in solution, behaves like one, and is therefore referred to as an admixture complex of an "amine+metallate salt". The organic-metallic complex may be present in a concentration from about 10 ppm to about 5% by wt in neutral or basic aqueous solution. In the lower range of this conc. up to about 2000 ppm, the complex is useful in aqueous process streams; in the higher range, from 2000 ppm to 5%, for a rinse for phosphated metal parts, in lieu of a conventional chromate rinse.

### DE3828489

This invention relates to a process for producing corrosion-inhibiting oxide layers on surfaces of structural elements consisting of steels or nickel-based alloys by hot-water oxidation of the structural elements for several hours in an aqueous medium, in particular for suppression of the radioactive contamination of the inside surfaces of primary circuits of water-cooled nuclear reactors. The object according to the invention is achieved in such a way that at least hydrated oxides, known per se, of metals of subgroup IV of the periodic table of the elements are released in the aqueous solution and the concentration of the metal compounds, which lead to the formation of these hydrated oxides, does not exceed the order of magnitude of 1 mu mol/l. It has been found that the hydrated oxides of extremely low solubility of some metals, above all of titanium and zirconium, in a particle size of less than 10 nm act as crystallization nuclei during the formation of the protective layer. They are also capable of penetrating into pores, which may already be present, having diameters of from 10 to 100 nm. The protection becomes effective in a total quantity, specific to unit area, of foreign metals in the order of magnitude from 0.1 g/m<2>, i.e. at only about 1/100 of the quantity hitherto used.

US3397150 describes using a composition including trichloro tri fluroethane to remove water from solid surfaces and prevent rusting of ferrous metal surfaces.

EP0818651 invention is particularly used for L.P.G. tank/ pipe application. It makes use of passivating agents which form a corrosive protective film on the surface.

GB 2 189 501 discloses anti-corrosion composition containing from 60 to 98%wt liquid of hydrocarbon filling material, from 1 to 30%wt of a corrosion inhibitor and from 1 to 10%wt of a gelling agent which at least in course of time gives the composition a viscosity of at least 560cSt. At 25°C, all weight percentages being based on the total of the filling material, corrosion inhibitor and gelling agent, suitable for use In pipe connectors in contact with sea water.

EP 0 651 074 discloses a method for inhibiting corrosion comprising incorporating Into an aqueous medium a water soluble corrosion inhibitor that comprises an N-ethosyx-20substituted imidazoline, the N-ethoxy substituent having from one to about thirty ethoxy units and the w-substituent being an unsaturated or polyunsaturated fatty chain of from about six to about thirty carbons.

GB 2 104 897 relates to a method of using corrosion inhibiters suitable for oil producing industry mainly applied for pipe line, tank of oil/gas, etc. It uses salt of amino amide and phosphate ester as corrosion Inhibitor. Amino amide is derived from amino alky piperazine converted to amino amide which is then reacted with carboxylic acid or amide derivative like fatty acid/fatty acid glyceride/ester/fatty acid chlorine. Phosphate ester is derived from reaction of phosphorylating agent with adduct such as phosphorous pentoxide etc. Alternatively it also uses phosphoramidate as a corrosion inhibitor.

US 3846071 discloses a cyclic amidine salt, where the salt moiety is an acidic phosphate ester of an oxyalkylated alcohol, either employed alone or in conjunction with a carboxylic acid, i.e. a binary cyclic amidine-oxyalkylated phosphate salt or a tertiary cyclic amidine-oxyalkylated phosphate-carboxylate salt and to uses for these salts particularly as corrosion inhibitors.

### DRAWBACKS IN PRIOR ART;

1. No standard method and compound available to remove the unsaturated oxide so as to arrest or control the growth rate of metal loss and corrosion.
2. The corrosion control or rust preventive oils do not attempt to quarantine the unsaturated oxide.
3. Films or layers formed on metal surface are more than 1 micron in thickness.
4. Quantity of the rust preventive oils to be applied is considerably more resulting in increase of costs.
5. As the unsaturated oxide is not quarantined the rate of corrosion restarts immediately thereby requiring repetitive treatment of the entire process of application at very less time intervals.
6. The methods or processes are curative rather than preventive in nature.

Object of the present invention, therefore, is removing the drawbacks or the deficiencies of the prior art thereby reducing the growth rate of corrosion and metal loss which is due to the primary oxide which forms at the time of manufacturing on the ferrous metal and its alloys,

Yet another object of the present invention is to develop a monolayer non-porous film of less than 1 micron with chemi-adsorbed organic compound bond to reduce the rate of corrosion at low very cost.

The foregoing objects of the invention are accomplished and the problems and shortcomings associated with prior art techniques and approaches are overcome by the present invention to reduce corrosion and prevent further metal loss.

Thus, It is the object of the present invention to dewater the metal surface, i.e. to remove the water of crystallization from the unsaturated oxides as such water of crystallization that inhibits ionization.

It is also the object of the present Invention to modify the crystal structure of unsaturated oxide, which In effect quarantines the unsaturated oxide for preventing subsequent growth rate of metal loss. This can be achieved only if chemical is donated to the metal surface by chemi-adsorption.

Accordingly the present invention provides a method of inhibiting corrosion on a metal surface comprising forming an organic compound by reacting at a temperature between 30 and 180C; a. an alcohol phosphate ester and multi-esters selected from the group consisting of mono, di, tri esters derived from a carbon chain below C16; b. a petroleum solvent selected from kerosene, mineral turpentine and/or its modified derivatives; c. a fatty amine and/or its block polymer; d. lanolin; and e. a colour and odour maintenance additive; and applying said compound to said metal surface.

In the preferred embodiment an organic compound is formed by a novel process comprising ascertaining the thickness of the layer of corrosion, selecting and mixing specific chemicals to give a synergistic effect so as to displace the primary embedded corrosion and modify the crystal structure of the unsaturated oxide by chemi-adsorption.

The present invention does not give an additional film that can be measured in microns but the collapse of the oxide cavity due to loss of water of crystallization results in reduction of corrosion. Saturated and Unsaturated oxides do not change its percentage on the surface of the metal but the draining of their water of crystallization accompanied by the change of the crystal structure results in the decrease In the rate of corrosion.

This modification of the crystal structure makes the oxides softer than their original form thereby loosing their anohoring on the metal surfaces.

The quantity of the compound so obtained and to be applied depends upon the thickness of the unsaturated oxide present on the metal surface. Depending on the application or the metal and the thickness of the oxide different solvent blends and different coupling agents can be used. Use of Lanoline also helps as a dewatering agent.

The formation of a homogenous and a bio degradable mass is a preferred embodiment of the present invention.

### WORKING OR EFFECT OF THE PRESENT INVENTION

The organic compound when applied to metal surfaces brings about the following:
a) Dehydration of water of crystallization from unsaturated oxides,
b) Modification of crystal structures of such unsaturated oxides thereby quarantining the oxide and making it docile,
c) Donating antistatic properties.

The unsaturated oxide has empty cavities holding water of crystallization as well as air pockets. On application of the said organic compound the unsaturated oxide looses its water of crystallization and its crystal structure gets modified.

The modified crystal structure of the unsaturated oxide, now being softer, collapses these empty cavities so as to form a mono film as a result of which the mother metal is isolated from the environmental donors such as oxygen, sulphor dioxide, Nitrogen, Carbon dioxide etc. Thus the unsaturated oxide gets quarantined, i.e. now there would be very limited scope for increase or decrease of oxide percentage.

Due to softer oxide conversion, the processing on metal surfaces becomes easier. The presence of high wetting properties forms a monolayer non-porous film, which is a milli-micron film, i.e., less than 1 micron, on the metal surface.

This helps In isolating embedded unsaturated oxides. Thus the process creates residual film thickness below 1 micron.

The process thus does not generate any anti-rust preventive film but the result is that the unsaturated oxide, which is embedded to the mother metal is made docile and it disassociates from the anchoring position and hence no external non-porous film is created.

The monolayer film itself develops anti-rust properties, which is not the same as applying an external layer like the anti-corrosive oils available in prior art. Thus it is an object of the present invention not to apply an external layer of any rust preventive oils as in prior art but to create a non-porous film, which is a result of the application of the present invention.

The quantity of the ingredients of the organic compound, obtained by the aforesaid process will depend upon the thickness of the unsaturated oxide on the metal surface to which the application is to be made.

Due to high wetting properties of the said organic compound, the milli micron, cavities can be easily penetrated. Hence this reduces the quantity of the organic compound required to be applied on the metal surface or minimizes the number of treatments to be made thereon.

A homogenous and biodegradable mass is obtained to form an organic compound to reduces corrosion and reduce metal loss.

The quantity of the said solvents is at least 50 % with a maximum of 90% of the entire mixture, the proportion of the said alcohol phosphate ester and multi-esters and fatty amines and/or its block polymer being in the ratio 9:1 out of the remaining mixture. The said alcohol phosphate ester, is selected from a group consisting mono, di, tri, esters derived from carbon chain below C16.

The said petroleum solvents and/or its derivatives are kerosene, mineral turpentine and/or its modified derivatives. The mental surface can be ferrous metals or its alloys. The said fatty amine derivative is used as a preservative. The Lanolin is also used as a dewatering agent to enhance adequate dewatering properties.

The thickness of the oxide layer is measured by means of a magnetic gauge.

An organic compound is obtained from the aforesaid process. A method of treating the metal surface with an effective and optimum corrosion-inhibiting amount of the said organic compound.

The formation of the modified crystal structure quarantines the unsaturated oxide. The quarantined unsaturated oxide forms a non-porous monolayer film on the metal surface. The thickness of the monolayer film is less than 1 micron. Further the said residual monolayer film has wetting properties.

### Example:

To illustrate the working of the present invention we are citing the following example. This example is just indicative and should not be considered to limiting to this example. The applications would vary according to the specific characteristics of the metal and thus this example cannot be construed to be exhaustive.

### Test method and equipments used:

◆ Test method used for cursory testing of each sample made is ASTM D-130 (which shows surface colour change so as to know the crystal structure has changed.
◆ Magnetic coat gauge is used to measure (saturated and unsaturated) oxide layer on the metal surface.
◆ Standard M.S. grade metal plates are used.
◆ Humidifier is used for environment testing.

### EXPERIMENT:

Three standard M.S.grade plates and three plates treated by spray method with excess drained from surface are kept for reaction for 24 hours at room temperature to get reddish colour change to gray or blackish colour.

Before treatment of two sets of metal plates Blank reading is taken by magnetic coat gauge. And after treatment also reading is taken. Then these two sets of treated and blank plates are kept in humidity chamber for one week and then for one week in open atmosphere for atmospheric corrosion donors.

Such six cycles are executed for reading.

### Results:

| **Ist Cycle:** | | | | |
|---|---|---|---|---|
| **Type of Sample** | **original micron Oxide** | **Cycles Micron oxide thickness** | **% growth of oxide w.r.t Std. Blank plate** | **% surface area covered** |
| Blank sample | 20 microns | 40 microns | 200% | 10% |
| Treated sample | 5 microns | 10 microns | -200% | 5% |

| **2nd Cycle:** | | | | |
|---|---|---|---|---|
| **Type of Sample** | **original micron Oxide** | **Cycles Micron oxide thickness** | **% growth of oxide w.r.t Std. Blank plate** | **% surface area covered** |
| Blank sample | 40 microns | 50 microns | 250% | 35% |
| Treated sample | 10 microns | 15 microns | -125% | 7% |

| **3rd Cycle:** | | | | |
|---|---|---|---|---|
| **Type of Sample** | **original micron Oxide** | **Cycles Micron oxide thickness** | **% growth of oxide w.r.t Std. Blank plate** | **% surface area covered** |
| Blank sample | 50 microns | 60 microns | 300% | 35% |
| Treated sample | 15 microns | 20 microns | 0% | 7% |

The formation of the modified crystal structure quarantines the unsaturated oxide. The quarantined unsaturated oxide forms a non-porous monolayer film on the metal surface. The thickness of the monolayer film is less than 1 micron. Further the said residual monolayer film has wetting properties.

### Example:

To illustrate the working of the present invention we are citing the following example. This example is just indicative and should not be considered to limiting to this example. The applications would vary according to the specific characteristics of the metal and thus this example cannot be construed to be exhaustive.

### Test method and equipments used:

◆ Test method used for cursory testing of each sample made is ASTM D-130 (which shows surface colour change so as to know the crystal structure has changed.
◆ Magnetic coat gauge is used to measure (saturated and unsaturated) oxide layer on the metal surface.
◆ Standard M.S. grade metal plates are used.
◆ Humidifier is used for environment testing.

### EXPERIMENT:

Three standard M.S.grade plates and three plates treated by spray method with excess drained from surface are kept for reaction for 24 hours at room temperature to get reddish colour change to gray or blackish colour.

Before treatment of two sets of metal plates Blank reading is taken by magnetic coat gauge. And after treatment also reading is taken. Then these two sets of treated and blank plates are kept in humidity chamber for one week and then for one week in open atmosphere for atmospheric corrosion donors.

### Conclusion:

Reading in growth rate of corrosion is stopped at 6^{th} cycle as standard blank sample covered 90% of the surface area. This result shows rate of corrosion is reduced by minimum 70% when said treatment is repeated 5 times.

The actual growth rate of treated plate as compared with blank plate comes to 14.2%.

### ADVANTAGES:

- The unsaturated oxide is quarantined, whereby there is no increase or decrease of oxide percentage.
- Due to softer oxide conversion, the processing on metal surfaces becomes easier.
- A residual mili-micron film, i.e. below 1 micron, on-metal surface is formed that helps in isolating embedded unsaturated oxides.
- The invention in the form of the compound can be used as a transit protector (shop primer).
- It dissociates unsaturated oxide molecules, which is easier to remove than those, which are embedded.
- The formation of a monolayer film that is less than 1-micron with high wetting properties of the compound reduces the quantity of the compound to be applied. This makes the product significantly cost effective.

## Claims

1. A method of inhibiting corrosion on a metal surface comprising:
forming an organic compound by reacting at a temperature between 30 and 180C;
a. an alcohol phosphate ester and multi-esters selected from the group consisting of mono, di, tri esters derived from a carbon chain below C16;
b. a petroleum solvent selected from kerosene, mineral turpentine and/or its modified derivatives;
c. a fatty amine and/or its block polymer;
d. lanolin; and
e. a colour and odour maintenance additive;
and applying said compound to said metal surface.

2. A method according to claim 1 wherein the quantity of said solvent is at least 50% with a maximum of 90% of the entire mixture, the proportion of said alcohol phosphate ester and multi-esters and fatty amine and/or its block polymer being in the ratio 9:1 out of the remaining mixture.

3. A method according to claim 1, wherein said metal surface is a ferrous metal or its alloys.

4. A method according to claim 1 wherein the compound forms a non-porous monolayer film on the metal surface.

5. A method according to claim 4, wherein the thickness of the monolayer film is less than 1 micron.

6. A method according to claim 4 wherein the monolayer film has wetting properties.

## Patentansprüche

1. Verfahren zur Korrosionsinhibierung auf einer Metalloberfläche, wobei das Verfahren folgendes umfasst:
das Bilden einer organischen Verbindung durch eine Reaktion auf einer Temperatur zwischen 30 und 180°C;
a) ein Alkoholphosphatester und Multiester, die aus der Gruppe ausgewählt werden, die Mono-, Di-, Triester, abgeleitet von einer Kohlenstoffkette unter C16, umfasst;
b) ein Petroleumlösungsmittel, das aus Kerosin, Testbenzin und/oder deren modifizierten Derivaten ausgewählt wird;
c) ein Fettamin und/oder dessen Blockpolymer;
d) Lanolin; und
e) einen Zusatzstoff zur Farb- und Geruchserhaltung;
und das Auftragen der genannten Verbindung auf die genannte Metalloberfläche.

2. Verfahren nach Anspruch 1, wobei die Menge des genannten Lösungsmittels mindestens 50 % und höchstens 90 % der gesamten Mischung beträgt, wobei das Verhältnis des genannten Alkoholphosphatesters und der Multiester und dem Fettamin und/oder dessen Blockpolymer bei 9:1 in der verbliebenen Mischung liegt.

3. Verfahren nach Anspruch 1, wobei es sich bei der Metalloberfläche um ein Eisenmetall oder dessen Legierungen handelt.

4. Verfahren nach Anspruch 1, wobei die Mischung einen nicht porösen Monoschichtfilm auf der Metalloberfläche bildet.

5. Verfahren nach Anspruch 4, wobei die Dicke des Monoschichtfilms geringer ist als 1 Mikron.

6. Verfahren nach Anspruch 4, wobei der Monoschichtfilm Benetzungseigenschaften aufweist.

## Revendications

1. Procédé pour inhiber la corrosion sur une surface métallique, comprenant les étapes consistant à :
former un composé organique par la réaction à une température comprise entre 30 et 180 °C ;
a. d'un ester de phosphate d'alcool et d'esters multiples choisis dans le groupe constitué par des mono, di, tri esters dérivés d'une chaîne de carbone inférieure à C16 ;
b. d'un solvant de pétrole choisi parmi le kérosène, l'essence de térébenthine minérale et/ou de ses dérivés modifiés ;
c. d'une amine grasse et/ou de son polymère séquencé ;
d. de la lanoline ; et
e. d'un additif de maintien de couleur et d'entretien ;
et appliquer ledit composé sur ladite surface métallique.

2. Procédé selon la revendication 1, dans lequel la quantité dudit solvant est d'au moins 50 % avec un maximum de 90 % de l'ensemble du mélange, la proportion dudit ester d'alcool de phosphate et esters multiples et amine grasse et/ou son polymère séquencé étant de 9:1 du mélange restant.

3. Procédé selon la revendication 1, dans lequel ladite surface métallique est un métal ferreux ou ses alliages.

4. Procédé selon la revendication 1, dans lequel le composé forme un film monocouche non poreux sur la surface métallique.

5. Procédé selon la revendication 4, dans lequel l'épaisseur du film monocouche est inférieure à 1 micron.

6. Procédé selon la revendication 4, dans lequel le film monocouche a des propriétés de mouillage.
